

## UNITED STATES PATENT OFFICE

2,014,343

## MANUFACTURE OF ARTIFICIAL FILAMENTS

Theodoor Koch and Johannes Gerardus Weeldenburg, Arnhem, Netherlands, assignors, by mesne assignments, to American Enka Corporation, Wilmington, Del., a corporation of Delaware

No Drawing. Application December 2, 1932, Serial No. 645,416. In Germany June 24, 1932

## 4 Claims. (Cl. 106—40)

Our present invention relates to a new method for producing filaments, threads and the like having a matt appearance or dull lustre from cellulosic solutions, especially from viscose or from cuprammonium cellulose solutions.

The adding of mixtures of non-volatile or difficultly volatile organic or inorganic substances and easily volatile organic substances to spinning solutions in order to produce artificial silk of reduced lustre is already known.

We have found that advantageous effects can be attained if tin oxide ( $\text{SnO}_2$ ) in combination with volatile organic substances is incorporated in a spinning solution, such as viscose or cuprammonium solution. As examples of volatile organic substances, which we preferably use, may be mentioned hydroaromatic cyclic oxy-compounds, such as cyclo-hexanol (hexahydrophenol  $\text{C}_6\text{H}_{11}\text{OH}$ ), methylcyclohexanol (hexahydro-dro cresol  $\text{C}_7\text{H}_{14}\text{O}$ ) or alicyclic alcohols of the group comprising fenchyl alcohol, terpenehydrate, terpineol, which may be used in the form of pine oil; but it should be understood that other easily volatile organic substances may be used.

The mixture to be added to the spinning solution according to the present invention has an exceptionally good covering power, so that degrees of mattness to the most varied extent can be achieved easily and even without large quantities of the solid substance, which otherwise adversely affects the resistance and structure, being necessary to be used. It is usually possible to manage with approximately 1% of tin oxide calculated on the artificial silk substance if the volatile additional substance be suitably selected. The pigment tin oxide is completely white.

In cases where viscose is used as a spinning solution a certain browning of the spun material can occur owing to the hydrogen sulphide developed in spinning and in the subsequent treatment on account of the partial formation of brown tin sulphide. This may occur especially in using precipitated tin oxide.

We have found that this evil can be avoided, if tin oxide, manufactured in a special manner, be used. It was particularly found that the tin oxide  $\text{SnO}_2$  produced by direct burning of the tin in oxygen is kept entirely inert in the viscose

and remains in a surprising manner quite white even in the treatment in the viscose process. The size of the particles of the tin oxide thus produced is very fine, so that a grinding is in many cases superfluous and the manufactured product can be mixed with the volatile organic additional substance by rubbing in without further treatment, and then can be emulsified or stirred in the spinning material, for example the viscose.

5

10

## Example

10 kilograms of viscose with 8% cellulose and 7% alkali are mixed with 8 grammes of tin oxide, which has been produced by burning the tin in oxygen. Thereupon 80 grammes of terpineol (so-called pine oil) is added and the mass stirred into homogeneous mixture. The viscose can, if necessary, be filtered and then spun in the usual spinning baths.

15

Instead of incorporating the added substances successively the tin oxide can be rubbed in with a smaller or larger quantity of pine oil and the paste then thoroughly stirred in the rest of the pine oil and the preparation thus produced is then emulsified in the viscose.

20

Having thus described our invention, what we claim is:

1. A spinning solution for the manufacture of soft-lustre, cellulosic products comprising a solution of the group consisting of viscose and cuprammonium cellulose, burnt tin oxide and a highly volatile, organic liquid.

30

2. A spinning solution for the manufacture of soft-lustre, cellulosic products comprising a solution of the group consisting of viscose and cuprammonium cellulose, burnt tin oxide and a volatile liquid of the group consisting of hydroxy-aromatic cyclic oxy-compounds, fenchyl alcohol, terpenehydrate, and pine oil.

35

3. A viscose spinning solution for the manufacture of soft-lustre, cellulosic products comprising approximately 10 kilograms of viscose, 7 per cent alkali, 8 grams of burnt tin oxide and 80 grams of pine oil.

40

4. A soft-lustre, cellulosic product containing burnt tin oxide.

45

THEODOOR KOCH.  
JOHANNES GERARDUS WEELDENBURG.